

## UNITED STATES PATENT OFFICE

2,270,979

## STEEL ALLOY

James H. Taylor, Detroit, Mich., assignor to  
Gorham Tool Company, a corporation of Michigan

No Drawing. Application January 24, 1935,  
Serial No. 3,268

4 Claims. (Cl. 75—12C)

This invention relates to ferrous alloys usable for cutting-tools and dies which must retain their hardness at high temperatures. More particularly, the invention relates to improvements in tool steels characterized by alloys of iron with molybdenum and carbon.

I have discovered that tool steels of the kind mentioned can be produced with highly superior qualities, in several respects, if boron be introduced into the alloy in appropriate proportions in accordance with this invention.

For illustration, I have found the following formula to be satisfactory:

|            | Per cent     |
|------------|--------------|
| Molybdenum | 8.50         |
| Chromium   | 4.00         |
| Cobalt     | 4.25 to 4.40 |
| Tungsten   | 1.50         |
| Vanadium   | 1.50         |
| Carbon     | 1.00         |
| Boron      | 1.00         |

Another practicable formula employs the first five elements above enumerated in the same proportions, with—

|        | Per cent |
|--------|----------|
| Carbon | .60      |
| Boron  | .75      |

A third practicable formula is like the second except that only .35% of carbon is used with the .75% of boron.

The above-named ingredients, in the respective proportions, when combined with the indicated percentages of iron (with the usual commercial content of other substances) produces a surprisingly high quality of steel appropriate for cutting-tools, dies and the like, in which the tendency to decarburization is remarkably reduced, the resistance to oxidation is increased, the degree of hardness is very high, and the cutting qualities and durability are considerably improved as compared with like alloys omitting the boron constituent. The described products are extremely satisfactory in forging and working.

My observation and tests demonstrate that typical alloys of iron and molybdenum and carbon, may be materially improved if a part of the normal carbon content is replaced by boron in approximately the illustrative proportions indicated.

A form of boron usable, for example, in the above formulae is boron carbide, which is approximately 80% boron and 20% carbon.

Among other advantages observable in tool steels produced in accordance with this inven-

tion, it is noteworthy that the incorporation of boron in the alloy materially reduces the tendency, usually typical of molybdenum steels, toward undesirable decarburization. It has been attempted, with some success, to combat that tendency by coating molybdenum steels with borax during fabrication and heat treatment, the borax coating serving to protect the metal more or less from the oxygen of the air. This borax coating process, however, is expensive and inconvenient; and it is rendered superfluous when, according to this invention, the proper proportions of boron are incorporated in the molybdenum steel alloys.

I am not prepared to assert definite reasons for the superiorities of the product resulting from the practice of this invention, but I am inclined, theoretically at least, to attribute the superior qualities, in part, to the supposition that the boron forms borides with other metals in the alloy, and that carbon and boron form a carbide of extreme hardness; the hardening of the matrix is perhaps attributable to grain refinement and change in space lattice on quenching the alloy from high temperature, and is accompanied by a certain amount of age hardening that occurs on heat treatment of alloys comprising sufficient proportions of molybdenum or tungsten or both. The resistance of my alloys to decarburization and oxidation is probably, but not certainly, due to the formation of thin, impervious coatings of oxides of boron and the other constituent metals which tend to exclude the oxygen of the air.

As will be evident to those skilled in the art, it is not essential to my invention that the precise proportions given in the illustrative formulae be employed or that the exact ingredients be used in all cases. On the contrary, my invention is susceptible of application to a considerable range of equivalents within the scope of the subjoined claims.

I claim:

1. An alloy steel comprising the following essential elements: carbon about .5% to .85%, molybdenum about 8.5%, chromium about 4% and boron about .3% to .5%; said steel having high speed properties and being characterized by stability against the formation of soft skin at forging and heat treating temperatures in ordinary atmospheres.

2. An alloy steel comprising the following essential elements: carbon not more than 1%, molybdenum about 8.5%, and boron not more than 1%; said steel having high speed properties and being characterized by resistance to the

formation of soft skin at heat treating temperatures in ordinary atmospheres.

3. An alloy steel containing carbon from .35% to 1.00%, molybdenum 8.50%, and boron in an amount not exceeding 1.00%, said steel being characterized by its resistance to decarburization at elevated temperatures in ordinary atmospheres.

4. An alloy steel containing carbon from .35% to 1.00%, molybdenum about 8.50%, and boron in an amount between about .75% and about 1.00%, said steel having high speed properties and being characterized by its resistance to decarburization at heat treating temperatures in ordinary atmospheres.

JAMES H. TAYLOR.